# EUROPEAN PATENT SPECIFICATION

(11) **EP 0 015 279 B1**
(45) Date of publication and mention of the grant of the patent: **13.04.1983**
(21) Application number: 79900757.0
(22) Date of filing: 14.06.1979
(51) Int. Cl.: C25D 11/22

(54) **COATING SYSTEM**
BESCHICHTUNGS-SYSTEM
SYSTEME DE REVETEMENT

(30) Priority: 28.06.1978 US 920053; 28.06.1978 US 920057; 26.12.1978 US 972928; 02.01.1979 US 22
(43) Date of publication of application: 17.09.1980
(73) Proprietor: Reynolds Metals Company, Richmond, VA 23235 (US)
(72) Inventor: DARROW, George R., Richmond, VA 23229 (US); WALSH, Adam J., Barrington, RI 02806 (US)
(74) Representative: Bass, John Henton
(86) International application number: US7900417
(87) International publication number: WO8000158

## Description

The present invention relates to a process for the production of colored protective coatings on articles of aluminum or aluminum alloys which have been previously anodized in a very special way in order to obtain products which are particularly suitable to be used in architectural applications.

There has been much time and attention devoted in the prior art to the production of aluminum articles in order to make them decorative or resistant to abrasion under atmospheric influence. Early processes have included coloring of aluminum articles which had previously been anodically anodized by the treatment of the same with dyes, such as aniline dyes. As the art is well aware, the thus resulting articles have poor resistance towards atmospheric influence. Other developments have included anodic oxidation of aluminum articles, followed by submersion in chemicals which penetrate into the pores of the oxide layer, so that when the thus treated aluminum article is placed in aqueous solutions of salts which also penetrate into the pores, combination with the first used chemical is possible. These processes have not proven practical for a wide variety of reasons.

It is also known in the prior art to simultaneously anodize and color aluminum articles. However, the art is aware that processes of this type result in only a limited selection of colors and that the processes are expensive and difficult to carry out and very rigid requirements are made for the working and heat treatment of the aluminum articles as the metallic structure therein is of the utmost importance for the result obtained. These simultaneous processes also demand the use of large currents and high voltages and consequent heavy refrigeration and are thus relatively expensive.

United States Patents 3,669,856; 3,769,180 and 3,849,263 represent recent developments in the field of coloring aluminum or aluminum al!oys. These patents are, in general, directed towards the coloring of anodized aluminum by immersing said article in a bath containing a salt of a particular metal and passing an alternating current between the previously anodized article and a counter- electrode.

Although the process of these patents represent a significant improvement in the field of coloring aluminum, nevertheless, no details are given as to how the previously formed anodic coating is formed on the aluminum and, in fact, at least the implication is present that conventional anodizing techniques are used.

It is also well known in the art of sulfuric acid anodizing of aluminum that two separate and distinct types of an oxide layer can be obtained which are generally referred to in the art as a hard coat or a non-hard coat. The conventional anodizing techniques utilized in the art result in the production of a non-hard coat. There are processes known in the art for the production of hard, dense anodic coatings, but the techniques employed in the art for the subsequent dyeing of these hard, dense coatings have involved the conventional immersion with a suitable dye, as opposed to an electrolytic coloring process. The reason for this might be due to the fact that the techniques for the production of hard anodized coatings result in the production of anodic layers which are significantly colored and can therefore only be dyed to darker, muddied colours by the use of organic or inorganic dyestuffs. The art is also aware that the thicker the anodic layer is formed that the darker the anodic layer will be and, in general, those processes which produced hard anodic layers had as one of their criticalities the production of a thick layer. These thick layers of anodic film are unsuitable for the novel process of this invention.

As has heretofore been stated, there are processes known in the art for the production of a hard anodized layer and these processes are generally referred to as low temperature (around 0°C or 32°F) processes, intermediate temperature (around 7°C or 45°F) and room temperature (around 21 °C or 70°F) processes. The hard coats which are produced via the low and intermediate temperature processes are unsuited for the use of the novel process of this invention for several reasons. In the first place, both processes are expensive and require substantial energy in order to be operative. Secondly, the use of both processes results in the production of a hard anodized coat having a relatively thick non-porous barrier layer which makes it difficult to colour electrolytically. Finally, both processes produce an anodized layer which is relatively thick (customarily 38 ,um-1.5 mil-or heavier) in order to obtain high heat resistance and is of a darkish, muddied colour, thereby rendering it unsuitable for use in a process where light, un- muddied colours are desired.

U.S. Patent 3,524,799 is directed towards a room temperature process for anodizing aluminum in order to produce hard, dense anodic coatings and the novel process of the present invention utilizes as one step thereof a modification of the process described by this patentee.

This patent describes the formation of hard, dense anodic coatings on aluminum or aluminum alloys by anodizing the aluminum in an aqueous electrolyte containing a mineral acid, such as sulfuric acid, a polyhydric alcohol of 3 to 6 carbon atoms and an organic carboxylic acid containing at least one reactive group in the alpha-position to the carboxylic acid group, such as lactic acid or glycine. In a preferred mode, the electrolyte also contains an alkali salt of a titanic acid complex of a hydroxy- aliphatic carboxylic acid containing from 2 to 8 carbon atoms, such as, for example, titanium di- lactate ammonium salt.

We have now discovered that the use of such anodizing techniques under specially selected conditions, but without the alkali salt of a titanic acid complex, provides extremely dense and hard anodic coatings optimally suited to architectural applications and that such anodized layers when colored using the techniques described in US Patent Nos. 3669856 and 3849263 provide aluminum and aluminum alloy surfaces of very pleasing, architecturally pure colors of exceptional uniformity. Additionally, the use of the combination of these prior art techniques apparently provides exceptionally throwing power in the coloring operation. Throwing power is a term of art defining the ability of a coloring bath and process to provide color uniformly to all surfaces of a workpiece undergoing coloring. Thus, a process and bath which demonstrates high throwing power provides uniform color to small creases, cracks, nooks, detents, etc., as well as the larger uniform surfaces of an aluminum or aluminum alloy workpiece being colored. High throwing power also permits the introduction into the coloring bath of a mix of workpieces in terms of their alloy composition and overall physical configuration to obtain uniform color of all such workpieces. In prior art coloring techniques it was often difficult, if not impossible, to obtain uniform coloring of workpieces of different alloys or shapes in a single colouring bath at the same time. Furthermore, it is well recognized by the skilled artisan in the aluminum colouring field, spacing of the various workpieces in the colouring bath was a critical factor in successfully uniformly colouring aluminum extrusions, particularly for architectural purposes. Such spacing restraints often required leaving sufficient distances between the individual pieces being coloured that substantial portions of the working volume of a given colouring tank were left empty during a colouring operation resulting in a very inefficient use of colouring tank capacity. The exceptional throwing power of the technique of the instant invention permits minimal spacing of the workpieces in the colouring bath and thus optimum usage of the colouring capacity of the colouring tank. This results not only in a more optimum efficiency in terms of use of tank capacity, but reduces substantially the chemical and power requirements of the electrolytic colouring process.

The present invention now provides a process for the production of coloured protective coatings on articles of aluminum or aluminum alloys wherein the article is first anodized and thereafter an alternating current is passed between the anodized article and a counter-electrode immersed in an acidic aqueous bath containing salts of metals capable of colouring the anodized layer, characterized in that the article is anodized in an electrolyte comprising from 12 to 24 weight percent sulfuric acid, from 1 to 4 volume percent of polyhydric alcohol of from 3 to 6 carbon atoms and from 1 to 4 volume percent of an organic carboxylic acid containing at least one reactive hydroxy, amino, keto or carboxyl group in the alpha-position in the absence of a titanic complex, at a temperature of 18-30°C (65-85°F) at a current density of 2.6-3.9 A/dm² (24-36 amperes/sq. ft.) until there is obtained an anodized layer having a thickness of from 5 to 2θµm (0.2 to 1.1 mils), prior to the colouring step.

In order to obtain the architecturally acceptable and desirable hard anodic coatings of pure clean colour as described above, it is absolutely critical that the anodic layer be from 5 to 28 µm in the thickness, and preferably 15 to 28 pm (0.6 to 1.1 mils), as opposed to the 25-127 pm (1-5 mils) set forth at column 3, line 26 of said U.S. Patent 3,524,799.

Apparently, as described in U.S. Patent No. 3,524,799 the combination is an anodizing bath of a polyhydric alcohol containing from 3 to 6 carbon atoms, and an organic carboxylic acid containing a reactive group in alpha-position to the carboxylic acid group will react with the hot reaction products formed during anodizing with or adjacent to the surface of the pore base, and thereby suppress the attack or dissolution of the forming oxide film by these products.

The mineral acid component of the electrolyte is sulfuric acid. The anodizing bath concentration of sulfuric acid is generally maintained between about 12% and about 20% by weight, preferably about 1 5%.

Polyhydric alcohols containing from 3 to 6 carbon atoms which may be employed in the practice of the invention, singly or in admixture, include glycerol, butane-diol 1,4-pentanediol-1,5 mannitol and sorbitol. The total amount of the polyhydric alcohol employed ranges from 1% to 4% by volume of the anodized electrolyte. The preferred polyhydric alcohol is glycerol at a concentration of between about 1% to about 2%.

The organic carboxylic acids containing a reactive group in alpha-position to the carboxylic acid group include acids in which the reactive group is hydroxy, amino, keto, or carboxyl. Examples of such acids include glycolic (hydroxyacetic), lactic (hydroxypropionic), malic (hydroxysuccinic), oxalic, pyruvic, and aminoacetic acids. Acyclic carboxylic acids such as lactic, malic, and glycolic amino-acetic (glycine) acids are preferred. Glycolic acid is specifically preferred in combination with glycerol. A mixture of two or more of these acids may be employed in combination with the mineral acid and the polyhydric alcohol. The amount of carboxylic acid included in the electrolyte is between 1% and 4% by volume of the bath. A preferred concentration when glycolic acid is used in combination with glycerol is between 1 and 2% by volume.

In order to achieve the results described above, the temperature at which anodizing is carried out must range from 18 to 30°C (65-85°F) with room temperature conditions, i.e. 20-24°C (68-75°F) being preferred.

In order to achieve the exceptionally hard and readily coloured anodic coatings, it is also necessary that the current density which is used in the anodizing operation be in the range of from 24 to 36 amperes/sq. ft. (2.6 to 3.9 A/d_{M}²).

The time required to achieve the desired film thickness of between 5 and 28 pm (0.6 and 1.1 mils) will vary with the other parameters of temperature, current density, chemical composition of the bath, etc., but generally anodizing times on the order of from about 8 to about 30 minutes produce acceptable results.

Following the special anodizing treatment, above-described, the aluminum article is thereafter colored electrolytically by passing alternating current between said article and a counterelectrode in an aqueous acidic solution containing a water soluble metal salt. The electrolytic coloring process is extremely well known in the art, and in this connection, is disclosed in the technical and patent literature, including U.S. Patent 3,669,856; 3,849,263 and 3,869,180; the disclosure of which is herein incorporated by reference. The preferred metallic salt is a salt of tin, although salts of nickel, cobalt, copper and silicomolybdic acid and silicotungstic acid can also be employed, individually or in combination. The salts of these metals could be formed by adding the metal to the sulfuric acid in the bath, but, preferably a sulfate salt of the metal is added to the bath for better control of the amount of the metal in solution in the electrolyte.

As is well known in the art, the metallic salts desired to provide the particular color can be utilized at a concentration of from 0.5 to 20% by weight, preferably about 2% by weight based on the electrolyte. The salts modify the pH of the electrolyte to which they are added, and the pH of the complete bath may ordinarily range from about 3.5 to 5. However, when the metallic salt is tin sulfate, the pH may be as low as 1, preferably 1.5. Tin in the preferred metal for the salt because of the high throwing power of the bath and resultant improved colour effects at such low pH values.

The alternating current may have a frequency of 10-500 periods per second, preferably 50 periods per second, and a voltage of 2-50 volts and a current density of 0.2-1.0 A/dm² based on the surface of the aluminum article. The counterelectrode which is employed is preferably made out of the same metal as the metal used in the electrolyte solution. Thus, for example, when utilizing a tin salt in order to impart a bronze color, it is preferred that the counterelectrode be made out of tin. As is known in the art, however, this is not necessary and counterelectrodes made of other materials, such as graphite, stainless steel or titanium can also be used.

It has been found that if the aluminum is anodized in the manner above-described and thereafter electrolytically colored in accordance with the teachings of U.S. 3,669,856 many significant advantages will be obtained as opposed to the use of conventional anodizing techniques. In the first place, the article which is obtained has a hard coating which makes it particularly adapted to be used in architectural applications. Additionally, the process of this invention permits the simultaneous electrolytic coloring of articles of varying sizes and shapes. This has been difficult if not impossible, to achieve in prior art processes due to the fact that uneven color was obtained when articles of different sizes and shapes were simultaneously electrolytically colored. Another advantage of the novel process of this invention resides in the fact that the aluminum article to be colored need only have electric contact at one edge thereof, as opposed to both edges. This results in a significant manpower savings. Another advantage of the novel process of this invention resides in the fact that it is possible to correct for too dark a color electrolytically which has heretofore been impossible with processes utilizing dyes or with processes involving simultaneous anodizing and coloring. According to this technique, after application of an excess of color the polarity of the coloring system is reversed and color can be subtracted from the anodized layer.

As has heretofore been stated, the electrolytic coloring process is carried out by passing an alternating current between the anodized article of aluminum or aluminum alloy which has been carried out in the manner above-described, and a counterelectrode immersed in an acid aqueous bath containing metal salts having coloring cations, wherein the colored tones of the coatings can be controlled in a simple manner by modulating the shape of the curve of the applied alternating voltage in such a manner that during the coloring process the alternating voltage will provide a suitable ratio between the two current directions for an advantageous transport of material and course of reaction with regard to said anodized aluminum article. The alternating voltage supplied is modulated as regarding its amplitude and/or frequency so as to make asymmetrical, thereby to control the color tone of the aluminum article. As is known in the art, the modulation of the alternating voltage can be carried out in several ways, such as simultaneously supplying two or more different alternating voltages or a superimposed direct voltage or by generating an alternating voltage having the desired frequency and curve shape.

The material for the counterelectrodes can be stainless steel, titanium, copper, nickel, but preferably tin because they lead to advantageously low energy consumption.

The strength of the alternating voltage in the modulation of the amplitude and/or frequency thereof according to the present process is from 5-50 volts, depending upon the composition of the electrolyte and the properties of the oxide layer previously formed. Preferably there is used a current density of from 0.1 to 0.5 A/dm², dependent on the electrolyte employed and a low treatment period of from 1 to 10 minutes.

As is known in the art, various soluble metallic salts can be employed. The preferred salts are those of tin, although salts of nickel, cobalt, copper, silicomolybdic acid and silicotungstic acid can also be employed. The electrolytic coloring bath also contains a strong acid which is desirably either sulfuric or hydrochloric.

As is well known in the art, the metallic salts, e.g., sulfates, chlorides, acetates, etc. desired to provide the particular color can be utilized at a concentration of from 0.5 to 20% by weight, preferably about 2% by weight based on the electrolyte. The pH of the electrolyte may vary considerably within the acid range, but pHs of about 1.5 have been found to be useful.

A particularly preferred embodiment resides in having present in the electrolyte a certain amount of aluminum. In this connection, the aluminum can be provided by the addition of suitable aluminum compounds, such as aluminum sulfate or a certain part of a previously used electrolytic bath can also be used. The amount of aluminum which is present in the electrolyte can range from 0-12 grams/liter, and more desirably, from 4-8 grams/liter.

As has heretofore been pointed out, the novel process of this invention is applicable to colour articles made from aluminum, as well as from aluminum base alloys of all kinds.

It is particularly preferred initially to supply a symmetrical alternating current and then add asymmetrical alternating current.

In addition, the colouring takes place faster, more efficiently if the alternating current is regulated relatively slowly of the order of a few seconds from 0 to the voltage which is desired for the colouring. This relates to both the starting up of the colouring and to a latter supply of another alternating voltage than the one initially used.

Further improvement in the throwing power of the colouring solution of the instant invention can be achieved by incorporation of material which serves as a complexing or sequestering agent for the colouring metal ion. Although the mechanism for this further improvement is not fully understood, it has been found that the addition of small amounts on the order of 5x10 to 5 x 1 0-3 grams/liter of, for example a combination of A-naphthol and gelatin in a ratio of about 2:1 naphthol to gelatin or 4,4 di(dimethyl-amino) diphenyl methane to the colouring bath provides even more improved colouring baths.

The following examples will illustrate the novel process of this invention, Examples 5, 7 and 8 being for the purposes of comparison only.

### Example 1

An aluminum article is anodised for about 24 minutes at 18°C (65°F) in an anodizing bath at 1.5 pH and having the following composition:

with a constant current density of about 2.6 amperes/sq. dm (24 amps/sq. ft.) and a DC voltage rising to about 20 volts. An anodic coating of about 20 µm (0.8 mils) is obtained. The anodized aluminum article is electrically connected with a counterelectrode of tin in an aqueous electrolyte containing 2% by weight stannous sulfate and about 50 ml concentrated sulfuric acid per liter, an alternating current at 5-8 volts is supplied to the electrodes at room temperature for a period ranging from 5-15 minutes and the current density is varied from 0.2 to 0.8 a/dm^{2.} Very attractive bronze tones or black are obtained on the aluminum articles, depending on the duration of the supply of alternating current.

### Example 2

The process of Example 1 is repeated with the exception that a deep red to black colour is obtained, depending on duration, using copper sulfate instead of tin sulfate, a pH of 4.0 and a counterelectrode of graphite.

### Example 3

The process of Example 2 is repeated with the exception that bronze tones to black are obtained using cobalt sulfate as the salt.

### Example 4

The process of Example 2 is repeated with the exception that bronze tones are obtained using nickel sulfate as the salt and a counter- electrode of nickel.

### Comparative Example 5

An aluminum article was anodized in accordance with normal anodizing techniques utilizing a current density of 2.6 amperes/sq. dm. (24 amps/sq. ft.) and an electrolytic bath comprising 20 weight percent sulfuric acid, and 8 grams/liter of oxalic acid. The temperature utilized ranged from 18-21 °C, and the resulting aluminum article had an anodized layer of 25 microns. The results produced was not suitable for colouring due to that fact that it was darkish in colour.

As is obvious from the above experiment, the anodizing solution used was other than that of the instant invention.

### Example 6

An aluminum article was anodized using a solution comprising 18 weight percent sulfuric acid, 1% glycolic acid and 1% glycerol. The anodizing was carried out at a current density of 3.9 amperes/sq. dm. (36 amps/sq. ft.) at a temperature of about 19.5°C. After 13 minutes an anodized layer of approximately 21.1 pm (0.83 mils) was obtained.

The anodized aluminum article was then electrolytically coloured by immersing the same into a bath comprising 25 grams/liter sulfuric acid, 22 grams/liter sulfonic acid, 25 grams/liter tin sulfate, 5 grams/liter aluminum sulfate, 0.2 grams/liter of A-naphthol and 0.4 grams of gelatin per liter. The electrolytic colouring was carried out by applying alternating current through the electrolyte at a voltage of 8 volts for three minutes. Three minutes of half-wave alternating current was then applied.

An aluminum article having a blackish colour was obtained.

### Comparative Example 7

An aluminum article was anodized utilizing the electrolyte solution of Example 6 at a current density of 4.3 amperes/sq. dm. (40 amps/sq. ft.) at a temperature of 20°C.

The anodized article which was obtained was thereafter electrolytically coloured in accordance with the techniques of the United States 3,669,856. This resulted in an article having poor colour.

### Comparative Example 8

An aluminum article was anodized utilizing the anodizing solution set forth in Example 6 at a temperature of 20°C and at a current density of 5.2 amperes/sq. dm. (48 amps/sq. ft.). The anodizing was carried out until an anodized layer was obtained which had a thickness of about 41.9 pm (1.65 mils). Subsequent colour anodizing of this material in accordance with the techniques of this invention resulted in spalling on the anodic film.

It is apparent that the thickness of the anodized layer obtained during the anodizing step was simply too great to produce the satisfactory product desired by the techniques of this invention.

### Example 9

An aluminum article was anodized utilizing the electrolyte solution of Example 6 at a temperature of 21 °C until an anodized layer having a thickness of about 20 pm (0.8 mils) was obtained.

This material was then electrolytically coloured utilizing the techniques of United States 3,669,856 and the colour solution of Example 6. Alternating current was applied for 11 2 minutes and thereafter a half-wave alternating current was applied for a half minute. The resulting material was coloured satisfactorily and was capable for use as an architectural material.

### Example 10

An aluminum article was anodized using the electrolytic solution of Example 6 at a temperature of 20°C for six minutes in order to obtain an article which had a thickness of approximately 10 µm (0.4 mils). This material was then electrolytically coloured utilizing the solution of Example 6 by passing normal AC current between the aluminum article and a counterelectrode for two minutes, thereafter an alternating current having a minus half-wave which was asymmetrical was applied for one minute.

A very acceptable black colour was obtained. It is to be noted that normal anodizing techniques could not have obtained colour in an anodic film this thin.

### Example 11

An aluminum article was anodized utilizing the solution of Example 6 at a temperature of 20°C, a current density of 3.9 amperes/sq. dm. (36 amps/sq. ft.) in order to obtain a material which had a thickness of 28 pm. The material was thereafter colour anodized utilizing the tin solution set forth in Example 6 and the technique of United States 3,669,856. Alternating current was applied for 11 2 minutes followed by half-wave at one minute. A perfectly acceptable coloured article was obtained.

### Example 12

The process of Example 9 is repeated with the exception that after the product was run to a bronze colour, it was immersed in an oxidizing acid, preferably 20-30 volume % nitric acid at room temperature, which resulted in a unfirm champagne colour. This colour is virtually impossible to produce in a uniform manner by any other known process.

The desirable hardness of coatings made in accordance with the invention is evidenced by high coating density. For example, four samples were prepared using 6063 alloy and the process of Example 9 except that the current times in the colouring bath were varied as follows, with the following results:

## Claims

1. A process for the production of colored protective coatings on articles of aluminum or aluminum alloys wherein the article is first anodized and thereafter an alternating current is passed between the anodized article and a counterelectrode immersed in an acidic aqueous bath containing salts of metals capable of coloring the anodized layer, characterized in that the article is anodized in an electrolyte comprising from 12 to 24 weight percent sulfuric acid, from 1 to 4 volume percent of polyhydric alcohol of from 3 to 6 carbon atoms and from 1 to 4 volume percent of an organic carboxylic acid containing at least one reactive hydroxy, amino, keto or carboxyl group in the alpha-position in the absence of a titanic complex, at a temperature of 18-30⁰C (65-85°F) at a current density of 2.6-3.9 A/dm² (24-36 amperes/sq. ft.) until there is obtained an anodized layer having a thickness of from 5 to 28 µm (0.2 to 1.1 mils), prior to the coloring step.

2. A process according to claim 1, characterized in that anodizing is performed at a temperature between 20 and 24°C (68 and 75°F).

3. A process according to claim 1 or 2, characterized in that the organic carboxylic acid is glycolic acid or lactic acid.

4. A process according to claim 1 or 2, characterized in that the polyhydric alcohol is glycerol.

5. A process according to claim 3 or 4, characterized in that the anodizing bath contains 1-2% by volume glycerol and 1-2% by volume glycolic acid.

6. A process according to any of claims 1 to 5, characterized in that the metal salt capable of coloring is a soluble salt of tin, nickel, copper, or cobalt.

7. A process according to claim 6, characterized in that the metal salt is a sulfate.

8. A process according to any of claims 1 to 7, characterized in that the coloring bath additionally contains an aluminum compound in a quantity of up to 12 grams, preferably 4 to 8 grams aluminum per liter.

9. A process according to any of claims 1 to 8, characterized in that an anodized layer of from 15 to 28 pm (0.6 to 1.1 mils) is formed prior to the colouring step.

10. A process according to any of claims 1 to 8, characterized in that alternating current of controlled asymmetry is employed in the coloring steps.

11. A process according to claim 10, characterized in that initially a symmetrically alternating voltage is passed followed by an asymmetrically alternating voltage.

12. A process according to claim 10 or 11, characterized in that the color in an already applied colored coating is corrected by reversing the polarity of the coloring bath.

13. A process according to any of claims 10 to 12 employing alternating current of controlled asymmetry in the coloring step, characterized in that the aqueous acid coloring bath also includes a sequestering agent for the metal salts.

14. A process according to claim 13, characterized in that the sequestering agent comprises a mixture of β-naphthol and gelatin or 4,4- bis(dimethylamino)diphenyl methane.

15. A process according to claim 13 or 14, characterized in that the sequestering agent is used at a concentration of between 5 x 10-⁵ to 5x 10-³ grams/liter of bath.

## Patentansprüche

1. Verfahren zur Herstellung von gefärbten Schutzbeschichtungen auf Gegenständen aus Aluminium oder Aluminiumlegierungen, wobei der Gegenstand zuerst anodisiert und danach zwischen dem anodisierten Gegenstand und einer in einem wässrigen, sauren, zur Fäbrung der anodisierten Schicht befähigte Metallsalze enthaltenden Bad eingetauchten Gegenelektrode ein Wechselstrom hindurchgeleitet wird, dadurch gekennzeichnet, dass der Gegenstand in einem Elektrolyt, der 12-24 Gew.% Schwefelsäure, 1-4 Vol. % mehrwertigen Alkohol mit 3-6 C-Atomen, und 1-4 Vol. % einer organischen Carbonsäure mit mindestens einer reaktiven Hydroxy-, Amino-, Keto- oder Carboxylgruppe in a-Stellung, in Abwesenheit eines Titankomplexes enthält, bei einer Temperatur von 18-30°C und einer Stromdichte von 2,6-3,9 A/dm² vor der Färbestufe solange anodisiert, bis eine anodisierte Schicht einer Dicke von 5-28 µm gebildet ist.

2. Verfahren nach Anspruch 1, dadurch gekennzeichnet, dass die Anodisierung bei einer Temperatur zwischen 20 und 24°C ausgeführt wird.

3. Verfahren nach Anspruch 1 oder 2, dadurch gekennzeichnet, dass die organische Carbonsäure Glykol- oder Milchsäure ist.

4. Verfahren nach Anspruch 1 oder 2, dadurch gekennzeichnet, dass der mehrwertige Alkohol Glycerin ist.

5. Verfahren nach Anspruch 3 oder 4, dadurch gekennzeichnet, dass das Anodisierungsbad 1-2 Vol.% Glycerin und 1-2 Vol.% Glykolsäure enthält.

6. Verfahren nach einem der Ansprüche 1-5, dadurch gekennzeichnet, dass das zur Färbung befähigte Metallsalz ein lösliches Salz von Zinn, Nickel, Kupfer oder Kobalt ist.

7. Verfahren nach Anspruch 6, dadurch gekennzeichnet, dass das Metallsalz ein Sulfat ist.

8. Verfahren nach einem der Ansprüche 1-7, dadurch gekennzeichnet, dass das Färbebad zusätzlich eine Aluminiumverbindung in einem Mengenanteil von bis zu 12 g/I, vorzugsweise 4-8 g/I, Aluminium enthält.

9. Verfahren nach einem der Ansprüche 1-8, dadurch gekennzeichnet, dass vor der Färbestufe eine anodisierte Schicht einer Dicke von 15-28 µm gebildet wird.

10. Verfahren nach einem der Ansprüche 1-8, dadurch gekennzeichnet, dass in den Färbestufen ein Wechselstrom kontrollierter Assymetrie verwendet wird.

11. Verfahren nach Anspruch 10, dadurch gekennzeichnet, dass anfänglich eine symmetrische Wechselspannung, gefolgt durch eine assymetrische Wechselspannung, hindurchgeleitet wird.

12. Verfahren nach Anspruch 10 oder 11, dadurch gekennzeichnet, dass die Farbe einer schon aufgebrachten gefärbten Beschichtung durch Umkehrung der Polarität des Färbebades korrigiert wird.

13. Verfahren nach einem der Ansprüche 10-12 unter Anwendung von Wechselstrom kontrollierter Assymetrie in der Färbestufe, dadurch gekennzeichnet, dass das wässrige, saure Färbebad auch ein Sequestrierungsmittel für die Metallsalze umfasst.

14. Verfahren nach Anspruch 13, dadurch gekennzeichnet, dass das Sequestrierungsmittel ein Gemisch von β-Naphthol und Gelatine oder 4,4-Bis-(dimethylamino)-diphenylmethan ist.

15. Verfahren nach Anspruch 13 oder 14, dadurch gekennzeichnet, dass das Sequestrierungsmittel in einer Konzentration zwischen 5×10⁻⁵ bis 5×10⁻³ g/I des Bades verwendet wird.

## Revendications

1. Procédé pour la production de revêtements protecteurs colorés sur des articles en aluminium ou en alliage d'aluminium selon lequel l'article est premièrement anodisé puis soumis à l'action d'un courant alternatif passant entre l'article anodisé et une contre-électrode immergée dans un bain aqueux acide contenant des sels de métaux capables de colorer la couche anodisée, caractérisé en ce que l'article est anodisé dans un électrolyte qui comprend de 12 à 24% en poids d'acide sulfurique, de 1 à 4% en volume d'alcool polyhydrique ayant 3 à 6 atomes de carbone et de 1 à 4% en volume d'un acide carboxylique organique contenant au moins un groupe réactif hydroxy, amino, keto ou carboxyle en position alpha en l'absence d'un complexe de titane à une température de 18 à 30°C (65 à 85°F) sous une densité de courant de 2,6 à 3,9 A/dm² (24 à 36 ampères/sq. ft.) jusqu'à ce qu'une couche anodisée soit obtenue ayant une épaisseur de 5 à 28 pm (0,2 à 1,1 mil), cette opération ayant lieu avant l'étape de coloration.

2. Procédé selon la revendication 1, caractérisé en ce que l'anodisation est effectuée à une température comprise entre 20 et 24°C (68 et 75°F).

3. Procédé selon la revendication 1 ou la revendication 2, caractérisé en ce que l'acide carboxylique organique est de l'acide glycolique ou de l'acide lactique.

4. Procédé selon la revendication 1 ou la revendication 2, caractérisé en ce que l'alcool polyhydrique est le glycerol.

5. Procédé selon la revendication 3 ou la revendication 4, caractérisé en ce que le bain d'anodisation contient 1 à 2% en vol. de glycerol et 1 à 2% en vol. d'acide glycolique.

6. Procédé selon l'une quelconque des revendications 1 à 5, caractérisé en ce que le sel de métal capable de colorer l'article est un sel soluble d'étain, de nickel, de cuivre ou de cobalt.

7. Procédé selon la revendication 6, caractérisé en ce que le sel de métal est un sulfate.

8. Procédé selon l'une quelconque des revendications 1 à 7, caractérisé en ce que le bain de coloration contient en outre un composé d'aluminium dans une teneur allant jusqu'à 12 gr, mais de préférence 4 à 8 gr d'aluminium par litre.

9. Procédé selon l'une quelconque des revendications 1 à 8 caractérisé en ce qu'une couche anodisée de 15 à 28 ^{p}m (0,6 à 1,1 mil) est formée avant l'étape de coloration.

10. Procédé selon l'une quelconque des revendications 1 à 8, caractérisé en ce qu'un courant alternatif d'asymétrie controlée est employé durant l'étape de coloration.

11. Procédé selon la revendication 10, caractérisé en ce que l'on fait passer tout d'abord une tension alternative symétrique puis une tension alternative asymétrique.

12. Procédé selon la revendication 10 ou la revendication 11, caractérisé en ce qu'après avoir appliqué le revêtement coloré, la couleur est corrigée par renversement de la polarité du bain de coloration.

13. Procédé selon l'une quelconque des revendications 10 à 12 dans lequel on emploie un courant alternatif d'asymétrie controlée lors de l'opération de coloration caractérisé en ce que le bain aqueux acide de coloration comporte également un agent de retenue pour les sels métalliques.

14. Procédé selon la revendication 13, caractérisé en ce que l'agent de retenue comporte un mélange de naphthol-β et de gélatine ou de 4,4-bis(dimethylamino)diphenilméthane.

15. Procédé selon la revendication 13 ou la revendication 14, caractérisé en ce que l'agent de retenue est introduit sous une concentration comprise entre 5×10⁻⁵ et 5×10⁻³ grammes par litre de bain.
